

## UNITED STATES PATENT OFFICE.

VICTOR NOAK HYBINETTE, OF JACKSON, MICHIGAN, ASSIGNOR TO HYBINETTE PATENTS CORPORATION, OF JACKSON, MICHIGAN.

## ANTIFATIGUE ALLOY.

No Drawing.

Application filed July 11, 1927. Serial No. 205,026.

My invention relates generally to metal alloys and more particularly to an aluminum alloy such as is disclosed in my co-pending application for U. S. Letters Patent filed 5 February 1, 1927, Serial No. 165,246, and in an application for patent filed by Victor Evers Hybinette on February 10, 1927, Serial No. 167,364; also in U. S. Letters Patent No. 1,579,481, issued April 6, 1926, to Victor Evers 10 Hybinette.

The object of my present invention is to provide an aluminum alloy that is characterized by having the desirable qualities of being anti or non-fatiguing and which result is attained by minimizing the proportions of certain of the metals entering into the alloy.

In my above mentioned co-pending patent application, and in the patent application and issued patent of Victor Evers Hybinette, 15 above mentioned, the alloy consists of aluminum, nickel and/or cobalt, metals of the chromium group such as chromium, tungsten, molybdenum and/or copper and/or manganese and/or magnesium and/or silicon, and

20 I propose to produce my anti-fatigue alloy in much the same manner as the aluminum alloys set forth in said applications and issued patent are produced, but in order to impart to the alloy the desired non-fatiguing 25 quality, I lessen the quantities of copper, magnesium and silicon that enter into the alloy.

I have found that in tests and experiments,

the alloys set forth in the above mentioned patent applications have exceptional advantages, due to their anti-fatigue qualities and 35 such desirable quality is enhanced by decreasing the copper, silicon and magnesium contents. I believe that this result is only what might be expected, for it is evident that the alloys containing relatively large amounts of 40 segregations do not have the non-fatiguing qualities to the same extent as alloys that are more on the order of solid solutions.

My improved anti-fatigue alloy consists mainly of aluminum, nickel and metals of 45 the chromium group, with manganese and/or other heavy metals containing about 0.20-0.50% each of copper, magnesium and silicon. In the production of my improved alloy, the same is quenched at about 50 900° F. and aged at from 200° to 400° F.

I claim as my invention:

1. A low fatigue alloy comprising at least 95% aluminum, nickel less than 2%, metals of the chromium group less than 1%, and less 55 than 0.50% of copper.

2. A low fatigue alloy comprising at least 95% aluminum, nickel less than 2%, metals of the chromium group less than 1%, and less than 0.50% each of copper, magnesium and 60 silicon, said alloy being quenched at about 900° F. and aged between 200° F. and 400° F.

In testimony whereof I affix my signature.

VICTOR NOAK HYBINETTE.